

## UNITED STATES PATENT OFFICE

2,495,757

LOW-METHOXYL POLYVALENT METAL  
PECTINATE FIBERS

Harry S. Owens, Berkeley, and Harry Lötzkar,  
Los Angeles, Calif., assignors to United States  
of America as represented by the Secretary of  
Agriculture

No Drawing. Application November 22, 1946,  
Serial No. 711,763

3 Claims. (Cl. 260—209.5)

(Granted under the act of March 3, 1883, as  
amended April 30, 1928; 370 O. G. 757)

1

This application is made under the act of March 3, 1883, as amended by the act of April 30, 1928, and the invention herein described and claimed, if patented, may be manufactured and used by or for the Government of the United States of America for governmental purposes without the payment to us of any royalty thereon.

This invention relates to the preparation of fibers from pectinic acids.

An object of this invention is to provide a process for preparing fibers composed of polyvalent metal salts of pectinic acids.

Another object of this invention is to provide fibers composed of polyvalent metal salts of pectinic acids.

These and other objects and advantages will be apparent from a description of the processes and products embodied in this specification.

It is of course well known that fibers can be made in the laboratory or plant. Many of these fibers are derived from cellulose. The fibers of this invention are derived from pectinic acids which in turn are derived from pectin. Pectin is produced in large quantities from citrus peel and apple pomace. From the pectin by a de-methoxylation procedure, low-methoxyl pectinic acids are made. For instance in U. S. Patent No. 2,358,430 to Willaman et al., September 19, 1944, is shown a method for de-methoxylating pectin by an enzymic hydrolysis. These low-methoxyl pectinic acids may also be prepared from pectin by alkaline or by acid hydrolysis.

Since there is considerable confusion with respect to naming the substances involved herein, it may be of interest to define some of the terms used. By "pectin" is meant the usual preparation of commerce extracted from various plant sources such as citrus peel or apple pomace without substantial de-methoxylation. By "peptic acid" is meant a substantially completely de-methoxylated pectin. By "pectinic acid" is meant a derivative of pectin with a methoxyl content intermediate between that of pectin and that of peptic acid.

The fibers of the instant invention are in the form of the salts of pectinic acids with polyvalent metals. In order to prepare these fibers an aqueous solution of pectinic acids, or a partially neutralized solution of pectinic acids, is extruded through an orifice into a suitable precipitating bath.

The following examples are illustrative of the invention:

## Example 1.—Zinc pectinate fiber

The pectinic acid used in this example contained 3.5% methoxyl and was prepared by en-

2

zymic de-methoxylation of pectin. A 1% solution of the pectinic acid was prepared by stirring the pectinic acid with the requisite amount of water and sufficient sodium hydroxide to give a final pH of 5.0. This partially-neutralized solution of pectinic acid was centrifuged to remove air bubbles and suspended matter, and then extruded through a nozzle having an opening 1 mm. in diameter into a bath of 1 normal solution of zinc chloride in 95% ethanol. The fiber so produced was soaked overnight in 70% ethanol and then stretched 47% by suspending the fiber and attaching a weight to the end thereof. The fiber was then dried and placed in an atmosphere of relative humidity 65% at 25° C. for 24 hours. The fiber which had a diameter of 0.015 mm. was found to have a tensile strength of 44,000 lbs./sq. in. The wet strength was found to be 9100 lbs./sq. in.

## Example 2.—Calcium pectinate fiber

Calcium pectinate fibers were prepared in manner similar to that set forth in Example 1. Thus a calcium pectinate fiber derived from pectinic acids (3.5% methoxyl content prepared by enzymic demethoxylation of pectin), spun in a 1 normal calcium chloride-95% ethanol bath, and stretched 44% had a diameter of 0.015 mm. and was found to have a tensile strength of 49,000 lbs./sq. in. This fiber when wet had a tensile strength of 9,000 lbs./sq. in.

## Example 3.—Calcium pectinate fiber

The pectinic acid used in this example had a methoxyl content of 3.0% and was prepared by alkaline de-methoxylation of pectin. A 1% solution of the pectinic acid was prepared by stirring with the requisite amount of water and sufficient sodium hydroxide to give a final pH of 4 to 5. The solution of partially neutralized pectinic acid was centrifuged to remove air bubbles and suspended matter and extruded through a nozzle having an opening 1 mm. in diameter. The precipitation bath was a 1 normal calcium chloride solution in water. The fiber was washed with very dilute (0.025 N) hydrochloric acid. This procedure yielded a good, continuous fiber composed of calcium salts of low-methoxyl pectinic acids.

## Example 4.—Calcium pectinate fiber

The process of Example 3 was repeated using as the precipitating bath a 1 normal solution of calcium chloride in water, adjusted to 0.2 normal with respect to hydrochloric acid. A continuous, strong fiber of calcium pectinate obtained.

*Example 5.—Calcium pectinate fiber*

A calcium pectinate fiber was prepared as described in Example 1 from a pectinic acid having a methoxyl content of 7.9% and prepared by enzymic de-methoxylation of pectin. The fiber was stretched 46% and had a diameter of 0.01 mm. and a tensile strength of 44,000 lbs./sq. in.

*Example 6.—Zinc pectinate fiber*

A zinc pectinate fiber was prepared as described in Example 1, from a pectinic acid having a methoxyl content of 7.9% and prepared by enzymic de-methoxylation of pectin. The fiber was stretched 56%, had a diameter of 0.011 and a tensile strength of 34,000 lbs./sq. in.

It has been shown above how to prepare the calcium and zinc pectinate fibers. In similar manner, other metal pectinate fibers can be produced. By merely changing the salt in the precipitating bath, other polyvalent metal pectinate fibers can be prepared. Thus in order to prepare copper, ferric, or chromium pectinate fibers, the bath should contain copper chloride, ferric chloride, or chromic chloride, respectively. If desired, mixtures of various polyvalent metal salts can be used in the bath to obtain a fiber of mixed polyvalent metal composition.

The fiber need not necessarily be stretched. However, it has been observed that in general stretching the fiber from 20 to 80% imparts considerable increase in the tensile strength of the fiber.

The dry tensile strength of the fibers herein disclosed has been found to vary from 20,000 to 70,000 lbs./sq. in. with an average strength of 40,000 lbs./sq. in. This obviously compares very favorably with the natural and synthetic fibers, for instance, wool which has a tensile strength of 21,000 to 38,000 lbs./sq. in. The wet strength of the polyvalent metal pectinate fibers is somewhat low being about 20% of the dry strength.

The concentration of pectinic acids in the spinning solution may be varied within fairly wide limits. Concentrations of from 1% to 8% have been found to give the best results. Pectinic acids of high molecular weight such as those prepared by enzymic de-methoxylation of pectin produce solutions which are too viscous to be handled readily and in using such pectinic acids, concentrations of about 5% are the maximum.

In order to bring the pectinic acid into solution and in order to get a solution liquid enough so that it can be spun, a small amount of sodium hydroxide or other alkali must often be added. Whether the alkali is necessary or not depends on the methoxyl content of the pectinic acid and the method by which it was prepared. If the pectinic acid was prepared by alkaline or acid de-methoxylation of pectin, no alkali is necessary if the methoxyl content is above about 5.0%. If, however, the methoxyl content is lower than about 5.0%, alkali must be added to bring the pectinic acids into solution. Enough alkali is added to bring the final pH to about 3.8 to 6.0. The pectinic acids prepared by enzymic de-methoxylation are much more insoluble than those mentioned above. In using pectinic acids made by the enzymic process, alkali must be added if the methoxyl content of the pectinic acid is lower

than about 8%. Again, sufficient alkali should be added to bring the pH to about 3.8 to 6. With those pectinic acids which are soluble enough in water to produce a solution, liquid enough to be spun, no addition of alkali is necessary.

The precipitating bath should be an aqueous solution of a polyvalent metal salt. It is preferred to have a considerable proportion of alcohol (or other water-soluble organic solvent such as isopropyl alcohol or acetone) present in this bath and thereby it will satisfactorily precipitate pectinic acids of any methoxyl content. Where the alcohol, or other solvent, is omitted, the bath will satisfactorily precipitate pectinic acids having a methoxyl content up to about 6%. The concentration of salt in the bath is not critical.

The process is applicable to pectinic acids having a wide range of methoxyl content from 3% to about 10%.

The fibers of this invention may be employed in any of the usual applications of natural and synthetic fibers, such as weaving or knitting textiles. The calcium pectinate fiber can be employed as a suture as it is non-allergenic.

The fibers can be dyed readily, more so than many natural and synthetic fibers. The polyvalent metal pectinate fibers can be dyed readily with acid dyes as there is a reaction between the metal cations and the acid dyestuff.

Cloth woven from the polyvalent metal pectinate fibers is much more fire-resistant than is cotton or rayon textiles.

Having thus described our invention, we claim:

1. An artificial fiber having a wet tensile strength of not less than about 9,000 pounds per square inch cross section comprising essentially a filament of calcium salt of a pectinic acid having a methoxyl content of 3 to 7.9%.

2. An artificial fiber having a dry tensile strength not less than about 20,000 pounds per square inch cross section comprising essentially a filament of a polyvalent metal salt of a pectinic acid having a methoxyl content of 3 to 7.9%.

3. An artificial fiber having a dry tensile strength not less than about 20,000 pounds per square inch cross section comprising essentially a filament of zinc salt of a pectinic acid having a methoxyl content of 3 to 7.9%.

HARRY S. OWENS.  
HARRY LOTZKAR.

## REFERENCES CITED

The following references are of record in the file of this patent:

## UNITED STATES PATENTS

|    | Number    | Name            | Date          |
|----|-----------|-----------------|---------------|
| 60 | 2,132,065 | Wilson          | Oct. 4, 1938  |
|    | 2,132,577 | Olsen et al.    | Oct. 11, 1938 |
|    | 2,155,361 | Myers           | Apr. 18, 1939 |
|    | 2,371,717 | Speakman        | Mar. 20, 1945 |
|    | 2,418,866 | Bryant          | Apr. 15, 1947 |
| 65 | 2,448,818 | McCready et al. | Sept. 7, 1948 |

## OTHER REFERENCES

Palmer et al., J. A. C. S., vol. 67 (1945), page 883; 1 page.